

Oct. 25, 1932.

W. MENDEL

1,884,069

METHOD OF FORMING COMPOSITE CORDS AND BRAIDS

Filed April 7, 1930



INVENTOR:

WILLIAM MENDEL,

*John E. Sarge*  
Hannay.

## UNITED STATES PATENT OFFICE

WILLIAM MENDEL, OF BEVERLY, NEW JERSEY, ASSIGNOR TO NEIDICH VISCOSE CORPORATION, OF BURLINGTON, NEW JERSEY, A CORPORATION OF DELAWARE

## METHOD OF FORMING COMPOSITE CORDS AND BRAIDS

Application filed April 7, 1930. Serial No. 442,397.

My invention may be advantageously employed to make filamentous materials which may be utilized in the production of ornamental textile fabrics, for instance, for the manufacture of hat crowns and trimmings.

The object and effect of my invention is to produce strings, threads, stranded cords, braids, etc., having the capacity for being brilliantly dyed which is characteristic of artificial textile filaments formed of cellulose acetate or cellulose nitrate, or similar cellulosic compounds, and with the greater tensile strength characteristic of natural textile filaments such as hemp, jute, flax, etc.

As hereinafter described, an essential feature of my invention is that such a natural filament or filaments, having the desired tensile strength, may be used as a core of the desired product, which is partially or completely covered with an artificial filament or filaments of such cellulosic material, twisted therewith or wrapped or braided thereon; such cellulosic covering material being subsequently subjected to the action of a solvent thereof to such a degree as to cause it to coalesce and adhere to its core. The latter effect may be enhanced by compressing the product, either before or after it is dried.

The product thus formed is characterized not only by greater tensile strength but by greater resistance to bending stresses than materials of the same size formed of either the natural or artificial materials employed in the composite product, and has the ornamental appearance of extremely lustrous straw.

My invention includes the various novel features of procedure and product herein-after more definitely specified.

In said drawing: Fig. I is a fragmentary enlarged perspective view of a cord wherein a single filament of covering material is twisted with a single filament of core material.

Fig. II is a cross sectional view of the structure shown in Fig. I.

Fig. III shows a fragment of the structure of Fig. I after the covering material has been subjected to the action of a solvent thereof.

Fig. IV is a cross sectional view, similar to

Fig. II, but showing the structure of Fig. III with the core material integrated with the covering material by the softening and deforming effect of the solvent of the latter.

Fig. V is a cross sectional view of the structure shown in Fig. IV but compressed and dried to form a substantially flat band or ribbon, wherein the core and covering materials alternate from edge to edge throughout its length.

Fig. VI is a fragmentary enlarged perspective view of a cord wherein a plurality of substantially straight core filaments are wrapped with a single filament of covering material.

Fig. VII is a cross sectional view of the structure shown in Fig. VI.

Fig. VIII shows a fragment of the structure of Fig. VI after the covering material has been subjected to the action of a solvent.

Fig. IX is a cross sectional view similar to Fig. VII but showing the structure of Fig. VI with the core material integrated with the covering material by the softening and deforming effect of the solvent of the latter.

Fig. X is a cross sectional view of the structure shown in Fig. IX but compressed and dried to form a substantially flat band or ribbon, wherein the core material is entirely sheathed by the covering material.

Fig. XI is a fragmentary enlarged perspective view of a braid wherein a plurality of core filaments are interlaced with a plurality of covering filaments.

Fig. XII is a cross sectional view of the structure shown in Fig. XI.

Fig. XIII shows a fragment of the structure of Fig. XI after the covering material has been subjected to the action of a solvent.

Fig. XIV is a cross sectional view similar to Fig. XII but showing the structure of Fig. XI with the core material integrated with the covering material by the softening and deforming effect of the solvent of the latter.

Fig. XV is a plan view of the structure of Fig. XIV compressed and dried to form a substantially flat band or ribbon wherein the core material is visible at intervals throughout the length of the fabric.

Fig. XVI is a cross sectional view of the braid shown in Fig. XV.

Referring to the form of my invention shown in Figs. I to V inclusive; the core 1 consists of a natural fiber or fibers of hemp or other material having the desired tensile strength. The covering material 2 is an artificial filament or filaments formed of a coagulated cellulosic compound such as cellulose acetate or cellulose nitrate. Said materials 1 and 2 twisted together as indicated in Fig. I form a composite cord 3, but the two materials are primarily separate and distinct, as indicated in Fig. II. Said composite product 3 is then immersed in or drawn through a liquid solvent of the artificial cellulosic material 2 but which has no solvent effect upon the natural material 1. If the material 2 is a product of cellulose acetate, it may be subjected to the action of ethyl acetate, or a mixture of alcohol and ether, both of which are suitable solvents for cellulose acetate. If the material 2 is a product of cellulose nitrate, acetone may be employed as the solvent. In any case, the effect of the solvent is to cause the cellulosic material 2 to coalesce upon and adhere to the natural core material 1, as indicated in Figs. III and IV, so that the cord 3 is then of substantially circular cross section as indicated in Fig. IV, and it may be dried in that form. However, either before or after it is dried, and preferably before it is completely dried, the cord 3 may be compressed to form a substantially flat band or ribbon, as indicated at 5 in Fig. V, conveniently by running said cord 3 between parallel rollers. In such flattened form the core 1 and covering material 2 alternate from edge to edge thereof through the length of the product 5.

In the form of my invention shown in Figs. VI to X inclusive, the core 7 is formed of a plurality of filaments of natural fibers such as above contemplated which, while in substantially straight parallel relation, are wrapped with a covering filament or filaments 8 of the cellulosic material aforesaid, to form the cord product 9. As indicated in Fig. VII, said core 7 and covering 8 are primarily separate and distinct. However, by subjecting them to the action of a solvent of the covering material 8, the latter is caused to coalesce upon the core material 7, and adhere thereto so as to form a substantially continuous sheath for the core material, as indicated in Figs. VIII and IX. As indicated in Figs. VII and VIII; the composite cord 9 is substantially round. However, either before or after it is dried, it may be compressed to form a substantially flat band or ribbon as indicated at 10 in Fig. X.

Referring to the form of my invention shown in Figs. XI to XV inclusive, the core 12 is a plurality of filaments of natural fibers such as above contemplated, which may be

arranged in parallel relation in a substantially common plane, as indicated in Fig. XII with covering filaments 13 of cellulosic material aforesaid, interlaced therewith by the operation of a suitable braiding mechanism 70 to form the substantially flat braid 14, in which the core material 12 and covering material 13 are separate and distinct, as indicated in Figs. XI and XII. However, by subjecting said braid 14 to the action of a 75 suitable solvent of the material 13, as above contemplated, said material 13 is caused to coalesce upon and adhere to the core material 12, as indicated in Figs. XIII and XIV.

The composite braid product shown in 80 Figs. XIII and XIV may be compressed either before or after it is dried, to a flatter band or ribbon 15, as indicated in Figs. XV and XVI, wherein the core material 12 is visible at intervals throughout its length. 85

As above noted, all of the composite products above described are capable of being more brilliantly colored, by ordinary dyes, than the natural textile fibers forming the cores thereof, and may be made like ordinary 90 thread or yarn suitable for being woven, knit, or otherwise utilized in textile fabrics. However, the products above described may be used singly in the formation of any suitable fabric. For instance, the braid shown in 95 Figs. XV and XVI has a sheen exceeding that of the most lustrous natural straw and may be formed of such width that successive convolutions thereof may be sewed together 100 to form a hat crown.

It is to be understood that the forms of my invention above described are merely typical, and that various modifications may be made therein without departing from the essential features of my invention, as defined in 105 the appended claims.

I claim:

1. The method of forming a stringlike structure, which consists in assembling natural and artificial filaments in a dry state, 110 and thereafter subjecting the structure to the action of a solvent of the artificial filament material until it coalesces and adheres to the natural filament material, and compressing said structure.

2. The method of forming a stringlike structure, which consists in assembling natural and artificial filaments in a dry state, and thereafter subjecting the structure to the action of a solvent of the artificial filament material until it coalesces and adheres to the natural filament material, and compressing said structure until the materials thereof are integrated, while the artificial material is 120 softened with the solvent.

3. The method of forming a stringlike structure, which consists in assembling natural and artificial filaments in a dry state, and thereafter subjecting the structure to the action of a solvent of the artificial filament 130

material until it coalesces and adheres to the filament material, entirely encircling the natural filament material, and compressing latter.

4. The method of forming a stringlike structure, which consists in assembling natural and artificial filaments in a dry state, and thereafter subjecting the structure to the action of a solvent of the artificial filament material until it coalesces and adheres to the natural filament material upon the exterior thereof, covering and concealing said natural material.

In testimony whereof, I have hereunto signed my name at Burlington, New Jersey, this 25th day of March 1930.

WILLIAM MENDEL.

70

5 10 15 20 25 30 35 40 45 50 55 60 65 70 75 80 85 90 95 100 105 110 115 120 125 130

material until it coalesces and adheres to the filament material, entirely encircling the natural filament material, and compressing latter.

5. The method of forming a stringlike structure, which consists in assembling natural and artificial filaments, in a dry state, and thereafter subjecting the structure to the action of a solvent of the artificial filament material until it coalesces and adheres to the natural filament material upon the exterior thereof, covering and concealing said natural material, and compressing said artificial material upon said natural material.

6. The method of forming a stringlike structure, which consists in assembling natural and artificial filaments, in a dry state, and thereafter subjecting the structure to the action of a solvent of the artificial filament material until it coalesces and adheres to the natural filament material upon the exterior thereof, covering and concealing said natural material, and compressing said artificial material upon said natural material until the structure is substantially flat.

7. The method of forming a stringlike structure, which consists in assembling natural and artificial filaments, in interlaced relation, in a dry state, and thereafter subjecting the structure to the action of a solvent of the artificial filament material until it coalesces and adhere to the natural filament material, and compressing said structure.

8. The method of forming a stringlike structure, which consists in assembling natural and artificial filaments, in interlaced relation, in a dry state, and thereafter subjecting the structure to the action of a solvent of the artificial filament material until it coalesces and adheres to the natural filament material, and compressing said structure until it is substantially flat.

9. The method of forming a composite structure, which consists in assembling soluble and insoluble filaments, in a dry state, and thereafter subjecting the structure to the action of a solvent of the soluble filament material until it coalesces upon, adheres to, and forms an outer coating upon the insoluble filament material.

10. The method of forming a composite structure, which consists in assembling soluble and insoluble filaments, in dry state, and thereafter subjecting the structure to the action of a solvent of the soluble filament material until it coalesces upon, adhere to, and forms an outer coating upon the insoluble